

# UNITED STATES PATENT OFFICE.

REINHOLD GRÜTER, OF CHARLOTTENBURG, GERMANY.

## VARNISH, LACQUER, OR THE LIKE AND PROCESS OF MAKING SAME.

1,195,673.

Specification of Letters Patent. Patented Aug. 22, 1916.

No Drawing.

Application filed November 15, 1913. Serial No. 801,292.

*To all whom it may concern:*

Be it known that I, REINHOLD GRÜTER, subject of the German Empire, residing at Charlottenburg, Germany, have invented 5 certain new and useful Improvements in Varnishes, Lacquers, or the like and Processes of Making Same, of which the following is a specification.

For the preparation of nitrocellulose-containing zapon varnishes, amyl acetate is almost exclusively used as the solvent. The varnishes prepared therefrom possess various disadvantages, which have created a desire for other solvents.

10 It has been found that excellent nitrocellulose- or celluloid-containing varnishes, lacquers, or the like can be obtained with the aid of esters of lactic acid in conjunction with hydrocarbons, and especially aromatic 15 hydrocarbons. These varnishes or the like obtained with the use of hydrocarbons show specially favorable properties. For example, varnishes made from lactic acid ester and alcohol give a rough, irregular or non- 20 uniform coating, this is not the case with the varnishes obtained with hydrocarbons and lactic acid esters; with these, smooth and uniform coatings are obtained. This advantage is particularly found in the case of aro-

25 matic hydrocarbons, but it also applies partially with the non-aromatic hydrocarbons, for example benzin. With the benzins, however, the solutions can not be diluted to so great an extent as with the aromatic hydro- 30 carbons. It has further been found that a greater amount of the aromatic hydrocarbons can be added to the solution of nitrocellulose in lactic acid esters than when one starts with amyl acetate as solvent. The

35 following comparative experiments show 40 this: If one dissolves five parts of nitrocellulose in 36 parts amyl acetate (parts in all cases means parts by weight) and then adds 78 parts of xylene, stirring well of course, 45 the nitrocellulose is partly precipitated again, and coatings made with such a solution are irregular or non-uniform. If the solution is allowed to stand it solidifies after some time to a thick, useless, gelatinous 50 mass. This occurs after a few days, according to the temperature. If, on the other hand, 5 parts of nitrocellulose are dissolved in 36 parts of lactic acid ester, for example ethyl lactate, and 78 parts of xylene are added, one obtains a thinly fluid, mobile solution

which does not show a separation or gelatinization either at once or after a long period of keeping.

It has even been found that the quantity of the aromatic diluent can be further considerably increased without the separation occurring which takes place with amyl acetate. For example, solutions have been made according to the following proportions of mixture: 5 parts nitrocellulose, 36 parts 60 ethyl lactate, 96 parts xylene; also 5 parts nitrocellulose, 36 parts ethyl lactate, and 114 parts xylene. The quantity of xylene can even be still further considerably increased without a separation taking place in the 65 varnish, lacquer or the like. Instead of the ethyl ester of lactic acid other esters of lactic acid can be employed, and instead of xylene the other aromatic hydrocarbons, as for example toluene and benzene can be employed. Also, mixtures of the different lactic acid esters, and likewise mixtures of the different hydrocarbons can be used. Besides these solvents or diluents, other solvents or diluents, such as usual for the preparation 70 of varnishes, lacquers or the like and are suitable for this purpose, can of course be also used within the ambit of the present invention.

It has also been found that the lactic acid 75 esters are excellent solvents for resins such as are used in the production of varnishes, lacquers and the like and are suitable for this purpose. Thus, for example, colophony, shellac, copals, and similar resins dissolve 80 readily, and one can thus in a similar way also prepare varnishes, lacquers, or the like containing besides the cellulose derivatives these resins or containing the latter alone. These substances may be generally referred 85 to as substances suitable for varnish purposes.

The new process is therefore of particular value, because by its aid it is possible to produce the varnish, lacquer, or like 90 solutions with great cheapness; for firstly the lactic acid esters are themselves cheap and, secondly, considerable quantities of aromatic hydrocarbons can be used with them, whereby the cost is still further reduced. 95 The possibility of using such large quantities of aromatic hydrocarbons is therefore particularly important, because the same are very cheap, the more so as these hydrocarbons do not need to be added in a pure state, 100 105 110

but one can also use mixtures of the different homologues, such as obtained as waste or by-products in the distillation of tar.

It has further been found that the lactic acid esters, are excellent solvents for the organic cellulose esters, and that upon the basis of the cellulose esters also it is possible to produce solutions and varnishes, lacquers, or the like possessing advantageous properties in the respect above mentioned. These solutions on the basis of the organic cellulose esters can also be produced even in high concentration, because the dissolving capacity of the lactic acid esters is also very great for the said cellulose esters. Likewise, as with celluloid, which, as is well known, is composed of nitrocellulose and camphor, the celluloid-like masses from acidyl celluloses also dissolve in lactic acid esters; in this case also considerable quantities of various resins, or other substances, may be added, for example camphor or camphor substitutes, such as are suitable for varnish purposes.

The solutions thus obtained may within a wide range have suitable diluents added to them. For many purposes it is preferable to use such diluents as do not mix with water, for example hydrocarbons, halogen carbon compounds, ethers, or mixtures of these bodies; also acetone and alcohols alone or mixed, for some purposes in admixture with the first mentioned diluents.

Examples: Solutions and varnishes, lacquers or the like can be made by bringing together the following quantities: 1. 10 part by weight of acetyl cellulose, 50 parts by volume of ethyl lactate, 30 parts by volume of benzene. 2. 10 parts by weight of acetyl cellulose, 50 parts by volume of lactic acid ester, 30 parts by volume of trichlorethylene, 20 parts by volume of alcohol. 3. 10 parts by weight of acetyl cellulose, 50 parts by volume of lactic acid ester, 50 parts by volume of chloroform. 4. 10 parts by weight of acetyl cellulose, 60 parts by volume of lactic acid ester, 20 parts by volume of absolute or commercial alcohol. 5. 10 parts by weight of acetyl cellulose, 40 parts by volume of lactic acid ester, 20 parts by volume of acetone. If it is desired to add resins to these solutions, these resins can first be easily dissolved in lactic acid ester and the desired amount of this solution can be added to the cellulose ester solutions. Such resin solutions may be obtained by dissolving one part by weight of copal of sandarac or colophony in two parts by weight of lactic acid ester, which can readily be done. Shellac also dissolves easily, but in this case it is of advantage to take somewhat more ester, for example, four parts of ester to one part of shellac.

Of the organic cellulose esters the acetyl cellulose is at present the most important; the cellulose esters of any other organic

acids may however equally well be taken, for example those of formic acid, benzoic acid and so forth. Also mixtures of these various cellulose esters can be taken and also mixtures of nitrocellulose and organic cellulose esters. Even cellulose esters which are more difficultly soluble in other solvents, as for example the aceto sulfates of cellulose, dissolve in lactic acid esters.

Instead of producing the solutions, lacquers, varnishes or the like in the cold they can be obtained with application of heat.

What I claim and desire to secure by Letters Patent is:—

1. A process for manufacturing solutions of varnishes or the like from the esters of cellulose, which consists in dissolving the said esters in a mixture of a lactic acid ester and hydrocarbons, and in the absence of large quantities of alcohol.

2. A process for manufacturing solutions of varnish or the like from the esters of cellulose, which consists in dissolving said esters in a lactic acid ester, and diluting the said solution with hydrocarbons.

3. A process for the manufacturing of solutions of varnishes or the like from the esters of cellulose, which consists in dissolving said esters in a lactic acid ester.

4. A process for the manufacture of solutions of varnishes or the like from nitrocellulose in a mixture of lactic acid ester and hydrocarbons.

5. A process for the manufacture of solutions of varnishes or the like from nitrocellulose, which consists in dissolving the nitrocellulose in a lactic acid ester.

6. A solution of varnish or the like, comprising an ester of cellulose dissolved in a lactic acid ester and a hydrocarbon, and free from large quantities of alcohol.

7. A solution of varnish or the like, comprising an ester of cellulose dissolved in an ester of lactic acid and having a hydrocarbon diluent.

8. A solution of varnish or the like, comprising nitrocellulose dissolved in an ester of lactic acid and a hydrocarbon.

9. A solution of varnish or the like, comprising nitrocellulose dissolved in a lactic acid ester, and having a hydrocarbon diluent, said solution being free from large quantities of alcohol.

10. A process for manufacturing solutions of varnishes or the like from the esters of cellulose, which consists in dissolving the said esters in a mixture of lactic acid ester and hydrocarbons, in the absence of large quantities of alcohol, and adding thereto substances suitable for varnish purposes, substantially as described and set forth.

11. A process for manufacturing solutions of varnishes or the like from the esters of cellulose, which consists in dissolving said

- esters in a lactic acid ester, and diluting the solution with substances suitable for varnish purposes, substantially as described and set forth.
- 5 12. A process for the manufacture of solutions of varnishes or the like and nitrocellulose, which consists in dissolving the said nitrocellulose in a mixture of lactic acid ester, and adding substances suitable 10 for varnish purposes, substantially as described and set forth.
13. A solution of varnishes or the like, comprising an ester of cellulose dissolved in a lactic acid ester and a hydrocarbon, and 15 free from large quantities of alcohol, and containing substances suitable for varnish purposes, substantially as described and set forth.
14. A solution of varnishes or the like, comprising an ester of cellulose dissolved in an ester of lactic acid, and containing substances suitable for varnish purposes, substantially as described and set forth. 20
15. A solution of varnish or the like, comprising nitrocellulose dissolved in an ester of lactic acid and a hydrocarbon, and containing substances suitable for varnish purposes, substantially as described and set forth. 25

In testimony whereof I have signed my name to this specification in the presence of two subscribing witnesses.

REINHOLD GRÜTER.

Witnesses:

HENRY HASPER,  
WOLDEMAR HAUPT.